

# United States Patent Office

3,018,291

1

**3,018,291**  
**N-DIALKYLAMINOALKYL ALKENYL**  
**SUCINIMIDES**

**SUCCESSIONS**  
Robert G. Anderson, Novato, Frank A. Stuart, Orinda, and Alan Y. Drummond, Richmond, Calif., assignors to California Research Corporation, San Francisco, Calif., a corporation of Delaware  
No Drawing. Filed Aug. 24, 1959, Ser. No. 835,400  
3 Claims. (Cl. 260—326.5)

This invention pertains to a new class of compounds particularly useful as lubricating oil addition agents. These new compounds are N-dialkyl-aminoalkyl alkenyl succinimides.

Alkenyl succinic anhydrides and numerous derivatives thereof are well known in the art. For example, alkenyl succinic anhydrides in which the alkenyl radical contains from 5 to 20 carbon atoms are taught as corrosion inhibitors in lubricating oil compositions. Also, products obtained by reacting such alkenyl succinic anhydrides with monoamines are taught as ferrous corrosion inhibitors for lubricating oil compositions.

However, the above known alkenyl succinimides are not useful as detergents in lubricating oil compositions. In contrast thereto, the alkenyl succinimides described herein are new compounds which are useful as detergents in lubricating oil compositions.

Thus, it is a primary object of this invention to present as new compounds, alkenyl succinimides which are particularly useful as detergents in lubricating oil compositions.

In accordance with this invention, we have discovered the new compounds, N-dialkylaminoalkyl monoalkenyl succinimides, are effective lubricating oil addition agents.

The N-dialkylaminoalkyl monoalkenyl succinimides of this invention are particularly effective as detergents in lubricating oil compositions. By the use of lubricating oil compositions containing these alkenyl succinimides, diesel and gasoline engine parts remain remarkably free of deposits and varnish even under severe operating conditions.

The new compounds of this invention, which are further described as N-dialkylaminoalkyl monoalkenyl succinimides wherein the alkenyl radical contains from 30 to 200 carbon atoms, and wherein said dialkyl amino alkyl radical contains a total of 3 to 10 carbon atoms can be represented by the formula:

2

where R is an alkenyl radical containing from 30 to 200 carbon atoms, R' is a divalent alkylene radical, and R<sup>2</sup> and R<sup>3</sup> are alkyl radicals. The sum of the carbon atoms in R', R<sup>2</sup> and R<sup>3</sup> is 3 to 10; that is, R', R<sup>2</sup> and R<sup>3</sup> contain a total of no more than 10 carbon atoms.

It is preferred that R is a polymer of an olefin containing from 2 to 5 carbon atoms, wherein the polymer has a molecular weight from 400 to 3000, more particularly from about 900 to about 1200. Such olefins 10 are exemplified by ethylene, propylene, 1-butene, 2-butene, isobutene, and mixtures thereof. Since the methods of polymerizing the olefins to form polymers thereof is immaterial in the formation of the new compound described herein, any of the numerous processes available 15 can be used therefor.

R' alkylene radicals include the divalent methylene radical, ethylene radical, propylene radical, butylene radical, etc. R<sup>2</sup> and R<sup>3</sup> alkyl radicals include methyl, ethyl, propyl, etc. It is particularly preferred that R' contains 3 carbon atoms, and that R<sup>2</sup> and R<sup>3</sup> each contain 1 carbon atom.

Amine reactants used in the formation of the poly-  
amine radical of the succinimide include dimethylamino-  
25 methylamine, dimethylaminoethylamine, dimethylamino-  
propylamine, dimethylaminobutylamine, dimethylamino-  
heptylamine, diethylaminomethylamine, diethylaminopro-  
pylamine, diethylaminoamylamine, dipropylaminopropyl-  
30 amine, methylpropylaminoamylamine, propylbutylamino-  
ethylamine, etc.

The preparation of the monoalkenyl succinimides herein can be described generally by the following equations, wherein a polyolefin is reacted with maleic anhydride, which is then reacted with a dialkylaminoalkylamine to form the desired monoalkenyl succinimide; using a polymer of isobutene as an example of the alkenyl radical, and using dimethylaminopropylamine to exemplify the dialkylaminoalkylamine.





2. The compound



wherein  $n$  is a number having a value of about 7 to about 50.

3. The compound of the formula:



wherein R is a polyolefin radical of from 30 to 200 car-

bon atoms which polyolefin is a polymer of an olefin of

from 2 to 5 carbon atoms, R' is a divalent alkylene radical of from 1 to 3 carbon atoms, R<sup>2</sup> and R<sup>3</sup> are alkyl radicals of from 1 to 3 carbon atoms, and R', R<sup>2</sup> and R<sup>3</sup> combined contain a total of no more than 10 carbon atoms.

## References Cited in the file of this patent

## UNITED STATES PATENTS

|           |                    |              |
|-----------|--------------------|--------------|
| 2,540,800 | Trigg et al. ----- | Feb. 5, 1951 |
| 2,638,450 | White et al. ----- | May 12, 1953 |

UNITED STATES PATENT OFFICE  
CERTIFICATE OF CORRECTION

Patent No. 3,018,291

January 23, 1962

Robert G. Anderson et al.

It is hereby certified that error appears in the above numbered patent requiring correction and that the said Letters Patent should read as corrected below.

Column 2, the end of the printed equation should appear as shown below instead of as in the patent:



Signed and sealed this 5th day of June 1962.

(SEAL)  
Attest:

ERNEST W. SWIDER

Attesting Officer

DAVID L. LADD  
Commissioner of Patents